# EUROPEAN PATENT SPECIFICATION

(11) **EP 0 340 250 B1**
(45) Date of publication and mention of the grant of the patent: **05.10.1994**
(21) Application number: 88906685.8
(22) Date of filing: 22.07.1988
(51) Int. Cl.: D06M 13/224, C10M 129/68, C07C 69/24, C07C 69/533, C07C 69/58

(54) **SPIN FIBER LUBRICANT COMPOSITIONS**
SCHMIERMITTELZUSAMMENSETZUNG FÜR SPINNFASERN
COMPOSITIONS LUBRIFIANTES POUR FILAGE DE FIBRES

(30) Priority: 06.08.1987 US 82769
(43) Date of publication of application: 08.11.1989
(73) Proprietor: The Lubrizol Corporation, Wickliffe, Ohio 44092 (US)
(72) Inventor: YODICE, Richard, Mentor, OH 44060 (US); LENTZ, Gregory, A., Twinsburg, OH 44087 (US)
(74) Representative: Crisp, David Norman
(86) International application number: US8802498
(87) International publication number: WO8901071

(56) References cited:
- FR-A- 1 336 631
- FR-A- 1 442 882
- GB-A- 1 492 052
- US-A- 3 177 143
- US-A- 3 464 922
- US-A- 3 575 856
- US-A- 4 103 068

## Description

This invention relates to the preparation of esters of neoalcohols and to the use of such esters as an additive in a spin fiber lubricant. More particularly, the invention relates to spin fiber lubricant compositions comprised of a liquid carrier and esterified neoalcohols of a particular defined structural formula.

Spin finish, spinning finish, dressing, treating agent, spinning lubricant, coating fiber finish, processing agent, textile treating agent, textile treating composition, conditioning agent--all of these terms are used to designate the same material: an antistatic lubricant applied to the surface of man-made fibers as soon as practical after the fiber has been formed. The properties of the applied material are dictated by several factors, among which are the fiber to which it is applied and the processing to which the fiber is to be subjected. In general, once the fiber has been converted into yarn and then into fabric, the role of the finish is complete; it is usually removed prior to or during dyeing.

Natural fibers have their own finish. Cotton, for example, has a wax coating. The crude material extracted from raw cotton fiber by chloroform, carbon tetrachloride, benzene, or other organic solvents is usually called wax. Presumably most of the wax is located in the cuticle, which lies on the outside of the fiber. Most cotton which is spun contains its natural wax. Dewaxed cotton does not spin well. The wax undoubtedly has desirable lubricating properties for spinning.

In the production of synthetic continuous filament yarns, it is necessary to apply to the filaments during the spinning operation a lubricating composition to reduce friction developed as the yarns pass over the metal and ceramic machinery surfaces. Since they are applied during the spinning step, they are frequently referred to as spin finishes. Such finishes usually contain a lubricating ingredient to reduce friction, an antistatic agent to reduce the build-up of static electrical charges on the surfaces of the yarn as it passes over various machinery components, an antioxidant or thermal stabilizing agent to reduce the build-up of resin deposits on the machinery and the yarn itself, and an emulsifying agent in order that the total system may be applied to the yarn from an aqueous emulsion.

The primary function of a finish is to provide surface lubricity to the yarn such that smooth high-speed transfer over various metallic guides can take place with a minimum of fiber breakage.

Finishes also bring about fiber to fiber cohesiveness which is necessary to maintain uniform diameter and uniform twist configurations in the continuous multi-filament yarn system and winding.

Most synthetic fibers, due to their hydrophobic nature, are static prone--that is, they demonstrate a marked tendency to retain electrostatic charges. During the processing of the yarn, high-speed operations accelerate generation and retention of electrostatic charges. Without static protection of yarn, several problems may occur thereto such as ballooning of yarn due to like charge repulsion between individual filaments, and tactile shock upon contact with processing equipment.

The electrostatic charges occurring on synthetic fibers may sometimes be disturbing to such a degree that they strongly impede or render completely impossible the further processing of the fibers.

To minimize wear and tear, heat damage, accumulation of static charges, and other like processing headaches, it has been found advantageous to enhance interfilament friction characteristics and fiber bundle cohesion generally by the use of finishes.

In preparation of yarns suitable for textile manufacture it is necessary to apply a lubricant to the filaments to permit processing of the yarn with minimum difficulty. As is well known in the art, selection of a suitable lubricant composition is not readily made, since many diverse requirements are imposed on the lubricant composition by the nature of a yarn's use and the manner in which it is manufactured. Of particular concern in high-temperature processing is the formation of hard insoluble resins and the fuming of the finish when contacting heated surfaces. Some earlier attempts at providing spin fiber lubricants are referred to below.

US-A-3,993,571 (Marshall, November 23, 1976) relates to yarn finishing for multifilament yarns used in food packaging. The preferred finishing composition comprises butyl stearate, sorbitan monoleate and polyoxyethylene (20) sorbitan monooleate.

US-A-3,827,114 (Crossfield, August 6, 1974) is directed to a synthetic fiber finish which provides improved processing performance, heat stability, and the like, and comprises a heat stable, hydrophilic antistat of an alkoxylated polyhydric alcohol fatty acid ester or an acylated alcohol ester; and a heat stable, hydrophilic emulsifier comprising an alkylene oxide condensate of polyhydric alcohols and/or long chain fatty acid esters or alkylene oxide condensates of an alkaryl hydroxy terminated compound.

US-A-4,049,766 (Eskridge, September 20, 1977) relates to a continuous spin-draw winding of nylon 6 to produce yarn filaments of mixed beta-alpha crystalline morphology. The improvement is wherein prior to drawing, a spin finish emulsion containing from about 0.1 to about 6% by weight of benzyl alcohol is applied to the filaments to enhance conversion of the beta uniformity of dye acceptance to the drawn filaments.

US-A-3,859,122 (Burks, Jr. et al, January 7, 1975) relates to improved feed yarn for draw-texturing that has a finish composed of about 55 parts by weight of an ester oil lubricant, about 45 parts of a nonionic surface active emulsifier, and about 0.6 to 2 parts of poly(oxyethylene-oxy-1, 2-propylene) glycol having a viscosity of about 9,000 SUS (1948 mm²/s). A preferred ester oil is di(tridecyl) adipate. A preferred emulsifier is a tetraoleate-laurate of a condensate of sorbitol with ethylene oxide, plus a small amount of a condensate of nonylphenol with ethylene oxide. Twist slippage and broken filaments are reduced to provide uniform textured yarn, and objectionable deposits on equipment are avoided.

According to one aspect of the present invention there is provided a spin fiber lubricant composition comprising
(A) a liquid carrier and
(B) at least one ester having the general formula
wherein R₁ is selected from an alkyl group containing 10 to 22 carbon atoms, an alkenyl group containing from 4 to 50 carbon atoms, an aryl group, an alkaryl and an aralkyl group, and R₂, R₃, and R₄ are each independently straight chain hydrocarbon groups, or branched chain hydrocarbon groups.

According to another aspect of the present invention there is provided a process for preparing a spin fiber lubricant additive which comprises reacting
(A) a neoalcohol having the structure wherein R₂, R₃ and R₄ are each independently straight chain hydrocarbon groups, or branched chain hydrocarbon groups, with
(B) an acid,

   R₁COOH

   or an anhydride derived therefrom,
wherein R₁ is selected from an alkyl group containing 10 to 22 carbon atoms, an alkenyl group containing from 4 to 50 carbon atoms, an aryl group, an alkaryl group and an aralkyl group.

We have now found it possible to provide a novel group of spin fiber lubricant compositions which include a liquid carrier having particularly defined ester compounds therein.

A feature of the invention is that the esters as well as the spin fiber lubricant compositions can be easily and economically manufactured.

An advantage of the present invention is that the spin fiber lubricant composition provides lubricating properties which are desirable for spinning materials.

Various preferred features and embodiments of the present invention will now be described by way of non-limiting example; reference being made to the accompanying general structural formula forming part hereof wherein like symbols refer to like molecular moieties throughout.

In order to clarify the following description of the spin fiber lubricant compositions of the invention individual components of the composition will be described. Thereafter, examples of such components will be put forth followed by specific examples of the compositions including some or all of the individual components.

It must be noted that as used in this specification and the appended claims, the singular forms "a", "an" and "the" include plural referents unless the context clearly dictates otherwise. Thus, for example, a reference to "a composition" includes mixtures of such compositions, reference to "an ester" includes reference to mixtures of such esters, and reference to "an emulsifying agent" includes mixtures of emulsifying agents and so forth.

Before describing the individual components of the invention, it should also be noted that the spin fiber lubricant composition is essentially comprised of the liquid carrier and the ester as defined further below. However, other embodiments of the invention include the liquid carrier, ester and an emulsifying agent. Further, the invention also includes material having thereon the fiber lubricant comprised of the liquid carrier and the ester as well as materials having thereon the fiber lubricant comprised of the liquid carrier, ester and emulsifying agent. Methods of utilizing the spin fiber lubricant compositions and the esters described herein are also disclosed.

### (A) Liquid Carrier

The purpose of the liquid carrier is to solubilize the ester of a neoalcohol. The preferred liquid carrier is water; however, if the ester is not water soluble, a liquid carrier consisting of oil may be used. The oil may be a mineral oil, vegetable oil or synthetic oil. Further, any carrier may be used with a solubilizer which increases the solubility of the ester in the carrier.

### (B) Neoalcohol Ester

The neoalcohol esters which are used in the composition in accordance with the present invention are compounds characterized by the structural formula (I)
wherein R₁ is a C₁₀₋₂₂ alkyl group, a C₄₋₅₀ alkenyl group, an aryl group, an alkaryl group or an aralkyl group, and R₂, R₃ and R₄ are each independently straight chain hydrocarbon groups, or branched chain hydrocarbon groups. The neoalcohol ester is made by the reaction of a neoalcohol with a carboxylic acid or anhydride or by transesterification of an ester with a neoalcohol. For example,
The neoalcohol ester is prepared by reacting equal equivalents of neoalcohol with equal equivalents of acid. However, in order to force the neutralization reaction to completion, an excess of the neoalcohol is employed. Normally, the neoalcohol is present in a 100% excess on an equivalent basis. Preferably, the neoalcohol is present in a 50% excess. The unreacted neoalcohol may be removed by distillation after the neutralization reaction is complete and reused for further neutralization reactions.

Normally, the neoalcohol and acid are added to a reaction vessel at room temperature. Stirring is begun and an acid catalyst is added to promote the reaction. The catalyst of choice is para-toluene sulfonic acid. Upon completion of the neutralization, the catalyst itself is neutralized with an appropriate base, such as aqueous sodium hydroxide.

The neoalcohol ester is normally formed at about 110°C, although it is preferred to conduct the reaction up to 150°C. The reaction further may be followed by monitoring the amount of water obtained.

As used in this specification and appended claims, the term "hydrocarbon" denotes a group having a carbon atom directly attached to the remainder of the molecule and having predominantly hydrocarbon character within the context of this invention. Such groups include the following:
(1) Hydrocarbon groups; that is, aliphatic (e.g., alkyl or alkenyl), alicyclic (e.g., cycloalkyl or cycloalkenyl), aromatic, aliphatic- and alicyclic-substituted aromatic, aromatic-substituted aliphatic and alicyclic groups, and the like, as well as cyclic groups wherein the ring is completed through another portion of the molecule (that is, any two indicated substituents may together form an alicyclic group). Such groups are known to those skilled in the art. Examples include methyl, ethyl, octyl, decyl, octadecyl, cyclohexyl, phenyl, etc.
(2) Substituted hydrocarbon groups, that is, groups containing non-hydrocarbon substituents which, in the context of this invention, do not alter the predominantly hydrocarbon character of the group. Those skilled in the art will be aware of suitable substituents. Examples include halo, hydroxy, nitro, cyano, alkoxy, acyl, etc.
(3) Hetero groups; that is, groups which, while predominantly hydrocarbon in character within the context of this invention, contain atoms other than carbon in a chain or ring otherwise composed of carbon atoms. Suitable hetero atoms will be apparent to those skilled in the art and include, for example, nitrogen, oxygen and sulfur.

In general, no more than about three substituents or hetero atoms, and preferably no more than one, will be present for each 10 carbon atoms in the hydrocarbyl group.

Terms such as "alkyl-based group", "aryl-based group" and the like have meaning analogous to the above with respect to alkyl and aryl groups and the like.

The hydrocarbon groups R₂, R₃ and R₄ may be alkyl groups containing from 1 to about 16 carbon atoms, preferably 1 to about 10 carbon atoms, and most preferably 1 to about 6 carbon atoms. Specific examples of alkyl groups of R₂, R₃ and R₄ includes methyl, ethyl, propyl, isopropyl, butyl, isobutyl, sec-butyl and t-butyl. Non-limiting examples of neoalcohols that may be employed in the practice of this invention are: 2,2-dimethyl-1-propanol, 2,2-dimethyl-1-butanol, 2,2-dimethyl-1-pentanol, 2,2-dimethyl-1-hexanol, 2,2-dimethyl-1-heptanol, 2,2-dimethyl-1-octanol, 2-methyl-2-ethyl-1-butanol, 2-methyl-2-ethyl-1-pentanol, 2-methyl-2-ethyl-1-hexanol, 2-methyl-2-ethyl-1-heptanol, 2-methyl-2-ethyl-1-octanol, 2,2-diethyl-1-butanol, 2,2-diethyl-1-pentanol, 2,2-diethyl-1-hexanol, 2,2-diethyl-1-heptanol, 2,2-diethyl-1-octanol, 2,2,3-trimethyl-1-butanol, 2,2,3-trimethyl-1-pentanol, 2,2, 3-trimethyl-1-hexanol, 2,2,3-trimethyl-1-heptanol, 2,2,3-trimethyl-1-octanol, 2,3-dimethyl-2-ethyl-1-butanol, 2,2,4-trimethyl-1-pentanol, 2,2,4-trimethyl-1-hexanol, 2,2,4-trimethyl-1-heptanol and 2,2,4-trimethyl-1-octanol.

The hydrocarbyl group R₁ is selected from alkyl, alkenyl, aryl, alkaryl and aralkyl groups. The alkenyl groups contain from 4 to 50 carbon atoms, preferably from 4 to 22 carbon atoms, and most preferably from 10 to 22 carbon atoms. Specific examples of alkenyl groups containing from 14 to 18 carbon atoms include the various tetradecenes, the various hexadecenes and the various octadecenes. The most preferred octadecene is 1-oleyl. The alkyl groups contain from 10 to 22 carbon atoms. Preferably R₁ is an alkyl group containing from 14 to 18 carbon atoms.

When R₁ is an aryl group the preferred hydrocarbyl groups are phenyl, alpha-naphthyl and beta-naphthyl.

When R₁ is an aralkyl group the preferred hydrocarbyl groups are alkyl-substituted phenyl, alkyl-substituted alpha-naphthyl and alkyl-substituted beta-naphthyl wherein the alkyl group is from 4 to 22 carbon atoms, and most preferably from 6 to 18 carbon atoms.

Non-limiting examples of carboxylic acids or anhydrides that may be reacted with neoalcohols are: lauric acid, myristic acid, palmitic acid, stearic acid, oleic acid, linoleic acid, linolenic acid, phenylacetic acid, benzoic acid, o-toluic acid, m-toluic acid, p-toluic acid.

The carboxylic acid or anhydride may be reacted with a neoalcohol in the presence of a catalyst such as para-toluene sulfonic acid. The course of the reaction may be followed by monitoring the amount of water of neutralization obtained. The neutralization may be conducted up to a temperature of 150°C. The catalyst may be neutralized with a base, and the reaction mass may be filtered to yield the product.

### (C) Emulsifying Agent

The composition of the present invention may further comprise (C) an effective amount of an emulsifying agent. The emulsifier of this invention may be an alkylene oxide adduct of an organic compound having an active hydrogen atom. Useful emulsifiers also function as lubricants.

Compounds suitable for use in preparing such adducts are fatty acids and fatty alcohols, preferably unsaturated, having 12 to 20 carbon atoms in their chains, polyhydric aliphatic alcohols and partial esters thereof, and alkyl phenols. Another class of suitable nonionic emulsifiers includes the partial fatty acid esters of polyols or their ethylene oxide adducts. As is known, ethylene oxide adducts have hydrophilic properties due to the ethylene oxide moiety, and when the other portion of the adduct is primarily hydrocarbon so as to provide a hydrophobic moiety, the compound can be expected to exhibit surface active properties. In general, ethylene oxide adducts containing a chain of at least at about 10 carbon atoms and at least three ethylene oxide units are useful in the practice of this invention. Preferably, the surface active adducts will contain at least about 10 ethylene oxide units in their molecules, since such compounds provide a composition with a high propensity for resisting the accumulation of electrostatic charges in addition to improving the manner in which the composition can wear the filaments. Preferred surface active agents are the adducts of ethylene oxide with a partial ester of fatty acids having at least 12 carbon atoms with polyols containing 3 to 6 hydroxyl groups, and the products obtained by esterifying an adduct of ethylene oxide and a polyol having 3 to 6 hydroxyl groups with a fatty acid having 12 to 22 carbon atoms. These products may be partial or complete esters and will preferably contain 20 to 50 ethylene oxide units in their molecules. A particularly preferred member of this class of surfactants is the material prepared by reacting one mole of sorbitol with about 30 moles of ethylene oxide and esterifying the product with about 5 moles of a 4:1 mixture of oleic and lauric acids, it is preferred to use a mixture of this surfactant with an alkylphenoxy polyoxyethylene ethanol which, preferably, is the product of about 5 or 6 moles of ethylene oxide with one mole of nonylphenol. The combination of small quantities of about 2 to 10% (percentages of finish ingredients herein are weight percentages based on the weight of non-aqueous finish ingredients), of this emulsifier with the sorbitol derivative surfactant performs excellently. It is essential that the emulsifiers fully emulsify the ester component of the finish in water. The emulsifier should be stable under conditions of use, i.e., it should have little tendency to smoke and form insoluble deposits when the yarn carrying the finish contacts hot surfaces.

The poly(oxyethylene-oxy-1,-2-propylene) diol of the present invention can be prepared as shown in US-A-2,425,845. Of the polyoxyalkylenes useful for this invention, the weight ratio of ethylene oxide groups, i.e., the groups (CH₂-CH₂-O), to propylene oxide groups, i.e., the groups
is between about 3:1 and 1:1 in order that the material remain fluid and water soluble. It is important that the viscosity of the polyoxyalkylene diol be between 5,000 and 50,000 SUS at 100°F (1082-10823 mm²/s at 37.8°C); preferably, its viscosity is about 9,000 SUS at 100°F (1948 mm²/s at 37.8°C). If the viscosity is too low, broken filaments of the yarn carrying the finish result; whereas, if the viscosity is too high, unwanted twist slippage in the draw texturing process occurs. It is also important that the finish contain not more than 5 percent, and preferably not more than 2 percent, of the diol component. If the finish contains more than about 5 percent, unwanted twist slippage occurs in the draw texturing process. Generally, if the viscosity of the diol is high, less is needed and vice versa.

The following examples illustrate the preparation of the ester of neoalcohols represented by formula (I). Unless otherwise indicated in the examples and elsewhere in this specification and claims, all parts and percentages are by weight, and all temperatures are in degrees Centigrade.

### EXAMPLE A

Add a mixture consisting of 100 grams (0.82 equivalents) brassylic acid (tridecanedioic acid) and 159.8 grams (1.23 equivalents) of 2,2,4-trimethyl-1-pentanol to a reaction vessel. Stir and heat while passing nitrogen through the system at 0.5 cubic feet per hour (4x10⁻⁶ m³/s). Add one gram of para-toluene sulfonic acid and heat the contents to 105°C. Collect about 10 milliliters of water in a Dean Stark Trap. Heat the contents to 150°C. Obtain the neutralization number (acidic) and add 50% aqueous sodium hydroxide to neutralize. Filter the contents and obtain the filtrate which should have a neutralization number (acidic) of about 1.5.

### EXAMPLE B

Following essentially the same procedure of Example A, 160 grams (0.47 moles) erucic acid (cis CH₃(CH₂)₇CH=CH(CH₂)₁₁COOH and 92 grams (0.71 moles) 2,2,4-trimethyl-1-pentanol are mixed and reacted. The neoalcohol ester obtained has a nil neutralization number (acidic).

### EXAMPLE C

Following essentially the same procedure of Example A, 190 grams (0.61 moles) behenic acid and 119 grams (0.91 moles) of 2,2,4-trimethyl-1-pentanol are mixed and reacted. The neoalcohol ester is obtained in 84% yield.

In one embodiment, the spin finish composition of the present invention comprises a concentrate of a two-component system of about 20-50% of the ester of a neoalcohol and 50-80% of a liquid carrier. Preferably, the ester is present at a level of 25-45% and the carrier at 55-75%, and most preferably, the ester is present at 30-40% and the carrier at 60-70%.

In another embodiment, the spin finish composition of the present invention comprises a concentrate of a three-component system of carrier, ester and emulsifying agent containing about 30-55% of the carrier, 30-50% of the neoalcohol ester and 15-25% of the emulsifying agent. Preferably, the carrier is present at 35-50%, the ester at 35-45% and the emulsifying agent at 15-25%. Most preferably, the carrier is present at 40%, the ester at 40% and the emulsifying agent at 20%, with all components at ±2%.

In one embodiment, the spin finish composition of the present invention comprises about 35-45 weight percent of a neoalcohol ester, 15-25 weight percent of an emulsifying agent and 35-50 weight percent of a carrier preferably in the form of coconut oil.

In applying the finishing composition of this invention to the filaments, e.g., nylon, conventional methods may be employed. In general, good results are obtained in both hot and cold drawing operations when the finishing composition is applied in amounts in the range of from about 0.2 to 1.5 percent and more preferably 0.8 to 1.0 percent by weight, based on the weight of the yarn. The finishing composition is desirably applied as an aqueous emulsion containing about 12 to 25 percent of the finishing composition. The finishing composition is applied to the yarn prior to drawing by conventional techniques which comprise, for example, bringing the yarn in contact with the composition while it moves during the course of production. The composition may be applied to the yarn by various methods and devices which may include use of a lubricating roll, wick, or having the yarn pass through a bath containing the finishing composition.

The following table shows examples of the spin fiber lubricant composition. Efforts have been made to ensure accuracy with respect to numbers used (e.g., relative amounts, temperature, etc.) but some experimental errors and deviation should be accounted for. Unless indicated otherwise, parts are parts by weight, temperature is in degrees centigrade, and pressure is at or near atmospheric. The table demonstrates the use of the spin finish of the present invention.

A polycaprolactam yarn (200 denier-32 filament) is prepared by conventional spin-draw techniques. Immediately after spinning the spin finish, in a three-component system, consisting of an ester of a neoalcohol, glycerol trioleate or an ethoxylated sorbitol ester of a mixture of oleic acid and lauric acid, and coconut oil is applied to the yarn at the rate of 0.1-2 weight percent based on the weight of the yarn and preferably 0.5 to 1 percent by weight of the yarn as 15 weight percent emulsion in water by means of a conventional kiss roll application.

In a two-component system where the spin finish consists of coconut oil and an ester of a neoalcohol, the spin finish is applied to the yarn at the rate of 0.2-2.5 weight percent based on the weight of the yarn and preferably 0.8 to 1.5 percent by weight of the yarn.

The composition of this invention may also be used with other agents such as anti-static agents, product stability agents, corrosion resistance agents, etc.

**Finish Compositions**

| Components | | Composition in Weight Percent | | | | | | |
|---|---|---|---|---|---|---|---|---|
| | | I | II | III | IV | V | VI | VII |
| Composition of Example | A | 40 | 40 | | | | | |
| | B | | | 40 | 38 | 35 | | |
| | C | | | | | | 42 | 40 |
| Glyceroltrioleate | | | 15 | 18 | | | 20 | 20 |
| EtO/sorbitol (30/1)m/[oleic acid/lauric acid (4/1)m] (1/5)m | | 15 | | | 20 | 20 | | |
| Coconut oil | | 45 | 45 | 42 | 42 | 45 | 38 | 40 |

## Claims

1. A spin fiber lubricant composition comprising
(A) a liquid carrier and
(B) at least one ester having the general formula
wherein R₁ is selected from an alkyl group containing 10 to 22 carbon atoms, an alkenyl group containing from 4 to 50 carbon atoms, an aryl group, an alkaryl group and an aralkyl group, and R₂, R₃, and R₄ are each independently straight chain hydrocarbon groups, or branched chain hydrocarbon groups.

2. The composition according to claim 1 wherein R₂, R₃ and R₄ are alkyl groups containing from 1 to 16 carbon atoms.

3. The composition according to claim 2 wherein R₂ and R₄ are methyl groups and R₃ is an isobutyl group.

4. The composition according to claim 1 wherein R₁ is an alkenyl group containing 17 carbon atoms.

5. The composition according to claim 1 wherein R₁ is an aryl group selected from phenyl, alpha-naphthyl and beta-naphthyl.

6. The composition according to claim 1 wherein the liquid carrier is selected from oil and water.

7. The composition according to claim 1 further comprising
(C) an effective amount of an emulsifying agent.

8. The composition according to claim 7 wherein the emulsifying agent is selected from an ethoxylated fatty alcohol; an ethoxylated fatty acid; an ethoxylated polyhydric alcohol; and an ethoxylated alkyl phenol.

9. A fibrous material having thereon the spin fiber lubricant composition according to claim 1 wherein the spin fiber lubricant composition is present on the material in an amount in the range of 0.1-2 percent by weight based upon the weight of the fibrous material.

10. A fibrous material having thereon the spin fiber lubricant composition according to claim 7 wherein the spin fiber lubricant composition is present on the material in an amount in the range of 0.2-2.5 percent by weight based upon the weight of the fibrous material.

11. A process for preparing a spin fiber lubricant additive which comprises reacting
(A) a neoalcohol having the structure wherein R₂, R₃ and R₄ are each independently straight chain hydrocarbon groups, or branched chain hydrocarbon groups, with
(B) an acid,
R₁COOH
or an anhydride derived therefrom,
wherein R₁ is selected from an alkyl group containing 10 to 22 carbon atoms, an alkenyl group containing from 4 to 50 carbon atoms, an aryl group, an alkaryl group and an aralkyl group.

12. The process according to claim 11 wherein R₂, R₃ and R₄ are alkyl groups containing from 1 to 16 carbon atoms.

13. The process according to claim 12 wherein R₂ and R₄ are methyl groups and R₃ is an isobutyl group.

14. The process according to claim 11 wherein R₁ is a alkenyl group containing 17 carbon atoms.

15. The process according to claim 11 wherein R₁ is an aryl group selected from phenyl, alpha-naphthyl and beta-naphthyl.

16. The process according to claim 11 wherein the equivalent ratio of neoalcohol to acid or anhydride is from 1:1 to 2:1.

17. The process according to claim 11 wherein the reaction of neoalcohol to acid or anhydride is conducted at a temperature from ambient up to 150°C.

18. The process according to claim 11 wherein the reaction of a neoalcohol with an acid is conducted in the presence of an acid catalyst.

## Patentansprüche

1. Schmiermittelzusammensetzung für Spinnfasern, umfassend
(A) einen flüssigen Träger und
(B) mindestens einen Ester der allgemeinen Formel
in der der Rest R₁ ausgewählt ist aus einem Alkylrest mit 10 bis 22 Kohlenstoffatomen, einem Alkenylrest mit 4 bis 50 Kohlenstoffatomen, einem Arylrest, einem Alkarylrest und einem Aralkylrest und die Reste R₂, R₃ und R₄ jeweils unabhängig voneinander unverzweigte oder verzweigte Kohlenwasserstoffreste sind.

2. Zusammensetzung nach Anspruch 1, wobei die Reste R₂, R₃ und R₄ Alkylreste mit 1 bis 16 Kohlenstoffatomen sind.

3. Zusammensetzung nach Anspruch 2, wobei die Reste R₂ und R₄ Methylgruppen sind und der Rest R₃ eine Isobutylgruppe ist.

4. Zusammensetzung nach Anspruch 1, wobei der Rest R₁ ein Alkenylrest mit 17 Kohlenstoffatomen ist.

5. Zusammensetzung nach Anspruch 1, wobei der Rest R₁ ein Arylrest ist, ausgewählt aus Phenyl-, alpha-Naphthyl- und beta-Naphthylresten.

6. Zusammensetzung nach Anspruch 1, wobei der flüssige Träger ausgewählt ist aus Öl und Wasser.

7. Zusammensetzung nach Anspruch 1, weiter umfassend
(C) eine wirksame Menge eines Emulgators.

8. Zusammensetzung nach Anspruch 7, wobei der Emulgator ausgewählt ist aus einem ethoxylierten Fettalkohol, einer ethoxylierten Fettsäure, einem ethoxylierten mehrwertigen Alkohol und einem ethoxylierten Alkylphenol.

9. Fasermaterial mit der aufgetragenen Schmiermittelzusammensetzung für Spinnfasern nach Anspruch 1, wobei die Schmiermittelzusammensetzung für Spinnfasern in einer Menge von 0,1 bis 2 Gew.%, bezogen auf das Fasermaterial, auf dem Material vorliegt.

10. Fasermaterial mit der aufgetragenen Schmiermittelzusammensetzung für Spinnfasern nach Anspruch 7, wobei die Schmiermittelzusammensetzung für Spinnfasern in einer Menge von 0,2 bis 2,5 Gew.%, bezogen auf das Fasermaterial, auf dem Material vorliegt.

11. Verfahren zur Herstellung eines Schmiermitteladditvs für Spinnfasern, umfassend die Umsetzung
(A) eines Neoalkohols der allgemeinen Formel in der die Reste R₂, R₃ und R₄ jeweils unabhängig voneinander unverzweigte oder verzweigte Kohlenwasserstoffreste sind, mit
(B) einer Säure der allgemeinen Formel
R₁COOH
oder ihrem Anhydrid,
wobei der Rest R₁ ausgewählt ist aus einem Alkylrest mit 10 bis 22 Kohlenstoffatomen, einem Alkenylrest mit 4 bis 50 Kohlenstoffatomen, einem Arylrest, einem Alkarylrest und einem Aralkylrest.

12. Verfahren nach Anspruch 11, wobei die Reste R₂, R₃ und R₄ Alkylreste mit 1 bis 16 Kohlenstoffatomen sind.

13. Verfahren nach Anspruch 12, wobei die Reste R₂ und R₄ Methylgruppen sind und R₃ eine Isobutylgruppe ist.

14. Verfahren nach Anspruch 11, wobei der Rest R₁ ein Alkenylrest mit 17 Kohlenstoffatomen ist.

15. Verfahren nach Anspruch 11, wobei der Rest R₁ ein Arylrest ist, ausgewählt aus Phenyl-, alpha-Naphthyl- und beta-Naphthylresten.

16. Verfahren nach Anspruch 11, wobei das Äquivalentverhältnis von Neoalkohol zu Säure oder deren Anhydrid von 1:1 bis 2:1 beträgt.

17. Verfahren nach Anspruch 11, wobei die Umsetzung von Neoalkohol mit Säure oder deren Anhydrid bei einer Temperatur im Bereich von Raumtemperatur bis 150 °C durchgeführt wird.

18. Verfahren nach Anspruch 11, wobei die Umsetzung eines Neoalkohols mit einer Säure in Gegenwart einer Säure als Katalysator durchgeführt wird.

## Revendications

1. Composition lubrifiante pour fibres à filer, comprenant
(A) un véhicule liquide et
(B) au moins un ester de formule générale
dans laquelle R₁ est choisi parmi un groupe alkyle contenant 10 à 22 atomes de carbone, un groupe alcényle contenant de 4 à 50 atomes de carbone, un groupe aryle, un groupe alkylaryle et un groupe arylalkyle, et R₂, R₃ et R₄ sont chacun, indépendamment, des groupes hydrocarbonés à chaîne droite, ou des groupes hydrocarbonés à chaîne ramifiée.

2. Composition selon la revendication 1, dans laquelle R₂, R₃ et R₄ sont des groupes alkyle contenant de 1 à 16 atomes de carbone.

3. Composition selon la revendication 2, dans laquelle R₂ et R₄ sont des groupes méthyle et R₃ est un groupe isobutyle.

4. Composition selon la revendication 1, dans laquelle R₁ est un groupe alcényle contenant 17 atomes de carbone.

5. Composition selon la revendication 1, dans laquelle R₁ est un groupe aryle choisi parmi les groupes phényle, α-naphtyle et β-naphtyle.

6. Composition selon la revendication 1, dans laquelle le véhicule liquide est choisi parmi l'huile et l'eau.

7. Composition selon la revendication 1, comprenant aussi
(C) une quantité efficace d'un agent émulsifiant.

8. Composition selon la revendication 7, dans laquelle l'agent émulsifiant est choisi parmi un alcool gras éthoxylé, un acide gras éthoxylé, un polyol éthoxylé et un alkylphénol éthoxylé.

9. Matière fibreuse sur laquelle se trouve la composition lubrifiante pour fibres à filer selon la revendication 1, dans laquelle la composition lubrifiante pour fibres à filer est présente sur la matière dans une proportion de 0,1-2% en poids, par rapport au poids de la matière fibreuse.

10. Matière fibreuse sur laquelle se trouve la composition lubrifiante pour fibres à filer selon la revendication 7, dans laquelle la composition lubrifiante pour fibres à filer est présente sur la matière dans une proportion de 0,2-2,5% en poids, par rapport au poids de la matière fibreuse.

11. Procédé de préparation d'un additif lubrifiant pour fibres à filer, qui comprend la réaction
(A) d'un néoalcool de structure dans laquelle R₂, R₃ et R₄ sont chacun, indépendamment, des groupes hydrocarbonés à chaîne droite, ou des groupes hydrocarbonés à chaîne ramifiée, avec
(B) un acide
R₁COOH
ou un anhydride qui en dérive,
où R₁ est choisi parmi un groupe alkyle contenant 10 à 22 atomes de carbone, un groupe alcényle contenant de 4 à 50 atomes de carbone, un groupe aryle, un groupe alkylaryle et un groupe arylalkyle.

12. Procédé selon la revendication 11, dans lequel R₂, R₃ et R₄ sont des groupes alkyle contenant de 1 à 16 atomes de carbone.

13. Procédé selon la revendication 12, dans lequel R₂ et R₄ sont des groupes méthyle et R₃ est un groupe isobutyle.

14. Procédé selon la revendication 11, dans lequel R₁ est un groupe alcényle contenant 17 atomes de carbone.

15. Procédé selon la revendication 11, dans lequel R₁ est un groupe aryle choisi parmi les groupes phényle, α-naphtyle et β-naphtyle.

16. Procédé selon la revendication 11, dans lequel le rapport des équivalents du néoalcool à l'acide ou à l'anhydride est de 1:1 à 2:1.

17. Procédé selon la revendication 11, dans lequel la réaction entre le néoalcool et l'acide ou l'anhydride est réalisée à une température allant de la température ambiante à 150°C.

18. Procédé selon la revendication 11, dans lequel la réaction entre le néoalcool et l'acide est réalisée en présence d'un catalyseur acide.
